

# United States Patent

Geisler

[15] 3,706,608

[45] Dec. 19, 1972

[54] **COMBUSTION TAILORING OF SOLID PROPELLANTS BY OXIDIZER ENCASEMENT**

[72] Inventor: **Robert L. Geisler, Lancaster, Calif.**

[73] Assignee: **The United States of America as represented by the Secretary of the Air Force**

[22] Filed: **March 24, 1970**

[21] Appl. No.: **24,894**

[52] U.S. Cl. .... **149/6, 149/5, 149/19, 149/20, 149/22, 149/42, 149/43, 149/44, 149/60, 149/61, 149/76, 149/85, 264/3 C**

[51] Int. Cl. .... **C06b 19/02**

[58] Field of Search..... **149/5, 8, 6, 19, 20, 22, 42, 149/43, 44, 60, 61, 76, 85; 264/3 C**

[56] **References Cited**

UNITED STATES PATENTS

|           |        |                   |       |
|-----------|--------|-------------------|-------|
| 2,982,640 | 5/1961 | Blake .....       | 149/8 |
| 3,120,459 | 2/1964 | Coates et al..... | 149/5 |

Primary Examiner—Carl D. Quarforth

Assistant Examiner—Stephen J. Lechert, Jr.

Attorney—Harry A. Herbert, Jr. and Cedric H. Kuhn

[57] **ABSTRACT**

Solid rocket fuel particles such as aluminum, beryllium, magnesium, or boron are encased in an oxidizer by crystallizing the oxidizer onto the fuel particles. Encasement of the fuel particles before binding with a binder matrix enhances the combustion efficiency of the propellant.

**3 Claims, 2 Drawing Figures**

PATENTED DEC 19 1972

3,706,608



Fig-1



Fig-2

INVENTOR.  
ROBERT L. GEISLER

BY *Harry A. Herbert*

ATTORNEY

## COMBUSTION TAILORING OF SOLID PROPELLANTS BY OXIDIZER ENCASEMENT

### BACKGROUND OF THE INVENTION

#### 1. Field of the Invention

This invention is in the field of solid rocket propellants.

#### 2. Description of the Prior Art

The mixing and casting of solid oxidizer particles and solid fuel particles in hydrocarbon binders to form a solid propellant grain is well known. It is also well known that, in order to burn efficiently, a solid propellant grain should combust in a smooth, layer-by-layer manner with combustion beginning at the surface of an opening running through its center and proceeding smoothly outwardly toward the case of the rocket motor.

In the prior art, oxidizer and fuel particles have been mixed into and contained by the binder matrix as discrete entities. Studies have shown that this results in propellant grains made up of relatively large oxidizer particles surrounded by pockets of smaller fuel particles within the binder matrix. Upon combustion, pockets of fuel particles exposed at the burning surface become rapidly heated, melt together, and exude as molten droplets onto the surface of the propellant. The molten droplets then roll around on the surface until several of them come together and form an agglomerate. Agglomerates thus formed are generally 10 to 100 times larger than the original fuel particles found in the pockets of unburned propellant grains. After formation, the agglomerates are transported into the combustion chamber by high velocity gaseous decomposition products formed by reaction between oxidizer and binder. During the process of agglomerate formation and transportation into the combustion chamber, from which they exit through the rocket nozzle, the fuel particles act as reducing agents and become oxidized as a result of reaction with oxidizer particles. The agglomerate formation process has been found to hamper the efficiency of the oxidation-reduction process. Further, the melting action prior to the formation of agglomerates leaves pits in the burning surface of the propellant grain which interfere with the smooth, layer-by-layer combustion necessary to obtain the highest combustion efficiency.

### SUMMARY OF THE INVENTION

It has now been found that combustion efficiency of solid rocket propellant grains is enhanced by crystallization of the oxidizer over the metal fuel prior to incorporation into the binder matrix. The incorporation, into the binder matrix, of oxidizer coated fuel particles enables the delivery of small fuel particles to the combustion zone without the melting and agglomeration process described above. Crystallization of oxidizer coats on to the surfaces of burn rate catalyst particles such as iron oxide may also be utilized in achieving propellants of ultra high burn rate.

### BRIEF DESCRIPTION OF THE DRAWING

FIG. 1 shows a cross section of a typical prior art propellant grain during combustion; and

FIG. 2 shows a cross section of a propellant grain contemplated by the present invention during combustion.

### DESCRIPTION OF THE PREFERRED EMBODIMENTS

This invention may be conveniently understood by viewing a cross section of a typical prior art solid propellant grain in conjunction with a cross section of a propellant grain of the type contemplated herein. FIG. 1 of the drawing is a cross section of a typical prior art propellant grain during the process of combustion. Oxidizer particles 1 and fuel particles 2 are shown as discrete particles within a binder matrix 3. During combustion, pockets of discrete fuel particles melt together to form larger single particles 4. Then, varying numbers of larger, melted together particles 4 roll around on the grain surface and form into agglomerates 5. High velocity gases created by reaction between the oxidizer and the binder carry the agglomerates away from the surface of the propellant grain into the combustion chamber proper where they are oxidized and blown out through the rocket nozzle. The agglomeration process lowers the efficiency of oxidation by lowering the surface area of fuel material exposed to the heat of the combustion chamber and in contact with oxidizer. Also, smooth layer-by-layer burning of the propellant is hampered when pockets of discrete fuel particles 2 melt together to form the larger single particles 4 leaving pits in the propellant grain surface.

In contrast to FIG. 1, FIG. 2 shows a propellant grain of this invention wherein, prior to being incorporated into the binder 3, the fuel particles 1 have been provided with a coat of oxidizer 2 by crystallizing oxidizer material on them. Coating of the fuel particles with oxidizer increases the efficiency of combustion of the fuel particles by insuring that the oxidation-reduction reaction between oxidizer and fuel takes place while the fuel particle is in its small, original size. For a given weight of fuel particles in a propellant grain, a greater amount of surface area is exposed for purposes of reaction by keeping the fuel particles discrete from one another with oxidizer coats than is accomplished by the prior art method described above. Further, coating fuel particles with oxidizer prevents the formation of pockets caused by the melting together of pockets of particles prior to agglomerate formation. Thus, more smooth, layer-by-layer burning is accomplished. Efficiency gains of from 2 to 10 percent may be obtained by coating the fuel particles as shown by FIG. 2 because the fuel is oxidized prior to its entry into the combustion chamber proper rather than being allowed to agglomerate.

Burn rate catalysts may also be coated with oxidizer to assist in the tailoring of combustion. Either burn rate accelerators such as iron oxide, iron blue, and copper chromate or burn rate decelerators such as oxamides, barbiturates, and guanadine derivatives may be coated with oxidizer and utilized to tailor the combustion rate as desired. Since coating places the accelerators or decelerators, whichever the case may be, in more intimate contact with the oxidizer, their action is made more effective at a given concentration level.

Examples of fuel particles and oxidizers which may be utilized in conjunction with one another according to this invention include such fuels as aluminum, beryllium, magnesium, and boron particles and such oxidizers as ammonium perchlorate, ammonium nitrate, cyclotetramethylenetrinitramine (HMX), cyclotrimethylenetrinitramine (RDX), and metal

perchlorates such as alkali metal perchlorates. Several methods are available for the crystallization of a solute onto a seed particle suspended in solution.

#### EXAMPLE I

Aluminum powder is placed in a saturated solution of ammonium perchlorate in water. The ammonium perchlorate is then shocked out of solution by rapidly lowering the temperature until a precipitate appears. The precipitate is a plurality of aluminum particle nuclei coated with ammonium perchlorate.

#### EXAMPLE II

Fuel particles such as boron, beryllium, and magnesium are substituted for the aluminum of Example I. Organic solvents such as dimethyl formamide, ethyl alcohol, and acetone are substituted for the water of Example I. In each case fuel particles coated with ammonium perchlorate result.

#### EXAMPLE III

Ammonium perchlorate coated fuel particles are obtained by dripping a nonsolvent, ethyl ether, into saturated solutions of ammonium perchlorate in the solvents of Examples I and II containing suspended fuel particles. The coated particles are then centrifuged and the liquid decanted.

#### EXAMPLE IV

Saturated solutions of ammonium nitrate, various alkali metal perchlorates such as sodium perchlorate or potassium perchlorate, HMX, and RDX are used in lieu of the ammonium perchlorate solutions of the previous examples and the methods of the previous examples utilized with similar results.

#### EXAMPLE V

Surface treatment of aluminum powder may be used to enhance the process of Example I. In this embodiment, aluminum powder is treated with perchloric acid to form a thin surface layer of the perchlorate derivative on aluminum. The resulting coated aluminum is then substituted for the nontreated aluminum powder of Example I and the method of Example I used to coat the treated aluminum.

Separation of oxidizer coated fuel particles from the saturated solutions of oxidizer may be accomplished either by centrifugal or sedimentation methods taking advantage of differences in specific gravity.

After preparing the oxidizer coated fuel particles of oxidizer coated burn rate catalysts, the coated particles

may be incorporated into a binder by standard propellant processing techniques. The binder, coated particles (either fuel, catalyst, or both), and any other additives may be charged into a standard horizontal or vertical propellant mixer and mixed at temperatures of from about 120°F to about 160°F. After mixing, the propellant is cast into molds or rocket motor cases with suitable mandrels and cured. Typical compositions which may be prepared are:

- 10      Binder—12 to 20% by weight  
        Oxidizer—60 to 75% by weight  
        Metal Fuel—0 to 20% by weight  
        wherein the binder may be hydroxy or carboxy terminated polybutadiene, a copolymer of butadiene with acrylic acid and/or acrylonitrile. The propellant may be plasticized with liquid hydrocarbon to improve processibility and mechanical properties. Either all or only part of the fuel may be oxidizer coated. Curatives may be added to the binder to achieve an infinite polymer network as is usual in the art.
- 15      I claim:  
        1. The method of tailoring solid rocket propellants comprising the steps of:  
            a. coating solid metal fuel particles with a crystallized coat of oxidizer selected from the group consisting of ammonium perchlorate, ammonium nitrate, metal perchlorates, cyclotetramethylenetetrinitramine and cyclotrimethylenetrinitramine;  
            b. mixing the oxidizer coated fuel particles with a binder material; and  
            c. curing the binder.  
        2. The method of tailoring solid rocket propellants comprising the steps of:  
            a. coating solid fuel particles selected from the group consisting of aluminum, beryllium, magnesium and boron with a crystallized coat of oxidizer selected from the group consisting of ammonium perchlorate, ammonium nitrate, metal perchlorates, cyclotetramethylenetetrinitramine and cyclotrimethylenetrinitramine;  
            b. mixing the oxidizer coated fuel particles with a binder material; and  
            c. curing the binder.  
        3. The method according to claim 2 wherein the binder is selected from the group consisting of carboxy terminated polybutadiene, hydroxy terminated polybutadiene, a copolymer of butadiene and acrylic acid, a copolymer of butadiene and acrylonitrile, and a terpolymer of butadiene with acrylic acid and acrylonitrile.

\* \* \* \* \*